

## UNITED STATES PATENT OFFICE

2,408,417

TANNING AGENTS AND METHODS OF  
TREATING HIDES AND SKINS THERE-  
WITH

William C. Ellenbogen, York, Pa.

No Drawing. Application April 15, 1944.  
Serial No. 531,294

7 Claims. (Cl. 8—94.26)

1

The present invention relates to the tanning of hides and skins, and particularly to tanning processes which employ as the tanning agent compounds or mixtures of compounds containing iron.

Various compounds or substances containing iron have been used for tanning purposes in the past, but in practically all cases the leather obtained was not very resistant to tearing nor stable on storing. Thus iron tanned leather tended to dry hard, and in general proved to be unsatisfactory when compared with vegetable- or chrome-tanned leather.

It is accordingly a primary object of this invention to provide a method of tanning with iron compounds which results in leather of good tensile strength and increased resistance to aging.

A further object of the invention is to provide improved iron-containing tanning agents which are capable of producing leathers having not only the above desirable properties but increased fullness and scuff resistance.

Still further objects and advantages of the invention will appear from the following description and appended claims.

The invention may be carried out by treating hides or skins with dilute aqueous solutions containing a ferric salt, a salt of a short chain mono or polycarboxylic acid having at least one hydroxyl group or of a polycarboxylic acid having at least one double linkage, and a salt of an amidine of a higher or long chain fatty acid. Prior to subjecting the hides or skins to the action of the above solutions for the purpose of tanning the same, the hides may be conditioned in the usual way, as for example, by dehauling, bating and pickling the same. It is also customary subsequently to fix the tan with a dilute solution of alkali bicarbonate or other equivalent alkali, after which the leather is tumbled and washed, and subjected to the usual treatment following tanning, such as fat liquoring, dyeing, drying and finishing. It is to be understood, however, that the invention is not to be limited to these customary procedures as applied either before or after the tanning.

In carrying out the tanning step as hereinbefore described any suitable ferric salt may be used, such as ferric sulfate, ferric chloride and ferric fluoride, or mixtures thereof. The mono or polycarboxylic acids which may be used in the form of their alkali salts include tartaric, citric, glycolic, malic, phthalic and maleic acids. As suitable amidines there may be used oleyl amidine, stearyl amidine, the amidine of palm

nut oil fatty acid, as well as derivatives of such amidines in which one or more of the hydrogen atoms attached to nitrogen is replaced with a straight or branched chain aliphatic radical. 5 The amidines are usually employed in the form of one of their addition salts, such as the chloride or sulfate, but in some instances it is possible to use the amidine per se, as when sufficient acid is furnished to the tanning solution from other sources or as a result of the treatment preliminary to tanning.

The following examples will further illustrate the nature of this invention and how it may be carried out in practice, but it is to be understood 10 that the invention is not limited to the details described therein, except as defined in the appended claims.

## Example I

One hundred pounds of sheepskins (pickled weight) which had been conditioned in the usual way prior to tanning, as by dehauling, batting, degreasing and pickling, were milled in an equal weight of a 5% salt solution for about 15 minutes. A tanning solution consisting of 12 pounds 20 of ferric sulfate, 6 pounds of sodium citrate and 1.5 pounds of the hydrogen chloride addition salt of oleyl amidine dissolved in sufficient water to make 8 gallons, was then added, after which the skins were tumbled in the resulting solution for about one and a half hours. Eight pounds of sodium bicarbonate were then added to the bath in small additions at intervals over a period of one hour. This fixed the tan. The leather was then tumbled for another half hour, after 25 which it was washed in water. It was then subjected to the usual steps following tanning, including fat liquoring, dyeing, drying and finishing.

## Example II

One hundred pounds of cow hide (lime split weight), which had been dehaired, limed and bated in the usual manner, were pickled for two hours in a solution consisting of 6 gallons of water, 2 pounds of 66° Bé. sulfuric acid and 9 pounds of common salt. A tanning solution consisting of 8 pounds of ferric sulfate, 4 pounds of sodium tartrate, 1 pound of the hydrogen chloride addition salt of oleyl amidine and 1 pound of caustic soda dissolved in sufficient water to make 5 gallons, was then added. The hides were tumbled in the resulting solution for about 30 2 hours. Six pounds of sodium bicarbonate were then added to the bath in small additions at intervals over a period of one hour, which fixed

the tan. The resulting leather was then fat liquored, dried and finished in the usual manner.

*Example III*

One hundred pounds of calf skin (pickled weight), which has been dehaired, limed, bated and pickled in the usual manner, were tanned by tumbling them for two hours in a tanning solution consisting of 8 pounds of ferric sulfate, 4 pounds of sodium glycolate and 1 pound of the hydrogen chloride addition salt of stearyl amidine dissolved in sufficient water to make 5 gallons. The resulting leather was then further treated and finished as described in Example I.

*Example IV*

One hundred pounds of steer bellies (pickled weight) which had been treated in the usual manner to prepare them for tanning, were tanned by tumbling them for two hours in a tanning liquor prepared by dissolving 12 pounds of ferric sulfate, 6 pounds of phthalic anhydride, 3.5 pounds of caustic soda, and 1.5 pounds of the hydrogen chloride addition salt of stearyl amidine in sufficient water to make 8 gallons. The resulting leather was then further treated and finished as described in Example II.

*Example V*

Four hundred pounds of cow hide (limed weight), which had been dehaired, limed and bated in the usual manner, were pickled in a solution consisting of 35 gallons of water, 4 pounds of 66° Bé. sulfuric acid and 32 pounds of common salt for about twenty minutes. The pickled hides were then tanned by tumbling them for two hours in a tanning solution prepared by dissolving 32 pounds of ferric sulfate, 10 pounds of cream of tartar, 6 pounds of caustic soda and 3 pounds of the hydrogen chloride addition salt of oleyl amidine in sufficient water to make 25 gallons. Twenty pounds of sodium bicarbonate were then added to the bath in small additions at intervals over a period of one hour, which fixed the tan. The leather was then tumbled for another half hour, after which it was washed in water, fat liquored, dried and finished in the usual manner.

The leathers obtained in accordance with the above examples were found to have a fine and smooth grain, and a full round feel. Moreover, they possess exceptionally high tensile strength and resistance to scuffing, and have very good aging characteristics substantially equal to, or even better in some instances than those of chrome-tanned leather.

The tanning solutions employed as described

herein may be prepared either by separately adding and dissolving the various ingredients constituting the active tanning agent, or by previously mixing these ingredients and then dissolving the mixture.

It is believed that the various constituents of the tanning solutions described herein interact, when dissolved, to form organic iron complexes which raise the precipitation point of the iron, thereby allowing proper penetration of the tanning agent into the hide. Regardless, however, of the way the materials interact in solution, they produce the above described desirable effects on the leathers tanned therewith.

Where mention is made herein and in the appended claims of oleyl amidine and stearyl amidine, it is to be understood that this has reference to the amidines of oleic and stearic acids respectively.

What I claim is:

1. A tanning agent comprising an iron salt, a substance selected from the group consisting of the salts of hydroxy mono and polycarboxylic acids and polycarboxylic acids having at least one double linkage, and a substance selected from the group consisting of the salts of amidines of higher fatty acids and derivatives of such amidines in which at least one of the hydrogen atoms attached to nitrogen is replaced by an aliphatic radical.

2. A tanning agent comprising ferric sulfate, sodium tartrate and a salt of oleyl amidine.

3. A tanning agent comprising ferric sulfate, sodium citrate and a salt of oleyl amidine.

4. A tanning agent comprising ferric sulfate, sodium tartrate and a salt of stearyl amidine.

5. The process of tanning hides or skins which comprises treating them with an aqueous solution containing an iron salt, a substance selected from the group consisting of the salts of hydroxy mono and polycarboxylic acids and polycarboxylic acids having at least one double linkage, and a substance selected from the group consisting of the salts of amidines of higher fatty acids and derivatives of such amidines in which at least one of the hydrogen atoms attached to nitrogen is replaced by an aliphatic radical.

6. The process of tanning hides or skins which comprises treating them with an aqueous solution containing a ferric salt, an alkali tartrate and a salt of an amidine of a higher fatty acid.

7. The process of tanning hides or skins which comprises treating them with an aqueous solution containing a ferric salt, an alkali citrate and a salt of an amidine of a higher fatty acid.

WILLIAM C. ELLENBOGEN.